

# UNITED STATES PATENT OFFICE.

JAMES E. HOLDER, OF GREEN LANE, PENNSYLVANIA.

## METAL ALLOY.

1,359,064.

Specification of Letters Patent. Patented Nov. 16, 1920.

No Drawing.

Application filed June 2, 1920. Serial No. 386,052.

To all whom it may concern:

Be it known that I, JAMES E. HOLDER, a citizen of the United States, residing at Green Lane, in the county of Montgomery and State of Pennsylvania, have invented 5 certain new and useful Improvements in Metal Alloys, of which the following is a specification.

This invention relates to improvements in 10 metal alloys, and the object is to provide an alloy that will adapt itself to general uses in the reduction or melting down of certain metals, used in the arts for different purposes, and the invention consists in combining 15 certain metals by means of a specified method, which will be described later, and in combining said metals in proportions that may differ under certain conditions, and when intended for use in different metallic 20 combinations.

The invention consists broadly in the method of combining copper and lead, in certain proportions, with any or all of the following, viz: iron, manganese and phosphorus, in relatively smaller proportions, by 25 the use of nickel and metallic arsenic.

The approximate proportions of the respective ingredients are as follows:

Lead, from 30 to 50 per cent.  
30 Copper, from 47 to 68 per cent.  
Nickel, from 1 to 5 per cent.  
Metallic arsenic, from  $\frac{1}{2}$  to  $1\frac{1}{2}$  per cent.  
Manganese,  $2\frac{1}{2}$  per cent.  
Phosphorus,  $\frac{1}{2}$  of 1 per cent.  
35 Iron,  $\frac{1}{2}$  of 1 per cent.

The proportions enumerated above are the approximate relative proportions and their ranges, as they will appear in the resultant product.

40 The method of carrying out my invention, is as follows:—

First an alloy is made of metallic arsenic and lead and this is poured into small ingots, for convenience in handling. Then, copper

and nickel are melted, under suitable cover, 45 and, when the copper and nickel are fluid, a certain portion of plain lead is added. The temperature of the mass is then brought to a high degree, and then the arsenical lead is added to the mass. 50

The entire mass is then well stirred, and then drawn, skimmed, and run into suitable molds.

The introduction of the iron, manganese and phosphorus is a matter that will be determined in each case, any or all of them being added to the mass at different times during the process, and the proportions while subject to variation are always relatively low, for the reason that these elements 55 are included principally for the toughening effect, and for the aid they supply in holding up the lead content.

What I claim is:—

1. A metallic compound containing lead, 65 copper, nickel, metallic arsenic, manganese, phosphorus and iron in the proportions specified.

2. A compound comprising lead, copper, nickel, metallic arsenic and a toughening 70 element in the proportions specified.

3. A compound containing lead from 30 to 50 per cent., copper from 47 to 68 per cent., nickel from 1 to 5 per cent., metallic arsenic from one-half to one and one-half 75 per cent., and phosphorus one-half of one per cent.

4. The method of forming a metallic compound, which consists of melting lead and metallic arsenic and forming it into ingots; 80 melting nickel and copper together and when fluid, adding thereto plain lead; raising to a high degree of temperature this mass and then adding the arsenical lead, stirring the entire mass and then running 85 it into molds.

In testimony whereof I affix my signature.

JAMES E. HOLDER.